# EUROPEAN PATENT APPLICATION

(11) **EP 3 766 650 A1**
(43) Date of publication of application: **20.01.2021**
(21) Application number: 20382645.8
(22) Date of filing: 17.07.2020
(51) Int. Cl.: B27N 1/00, B27N 1/02, B27N 3/00, B27N 3/04

(54) **METHOD FOR THE PRODUCTION OF ARTIFICIAL WOOD BOARD**

(30) Priority: 17.07.2019 ES 201930660
(71) Applicant: Greenpoint Natura, S.L., 30007 Murcia (ES)
(72) Inventor: SANCHEZ IMBERNON, MANUEL ANGEL, 30007 MURCIA (ES); RUBIO ALEMAN, JOSE LUIS, 30007 MURCIA (ES)
(74) Representative: Isern Patentes y Marcas S.L.

(57) **Abstract**

The present invention relates to a mixture comprising natural coconut husk coir particulate and/or balsa wood particulate and an adhesive. The present invention also relates to a construction board comprising said mixture and to the method of preparing the mixture and the construction board.

## Description

### Field of the invention

The present invention relates to a mixture of natural coconut husk coir particulate and/or balsa wood and/or ground algae for manufacturing products.

### State of the art

In recent years, society has been placing enormous importance on the use of recycled materials and natural materials which can be readily recycled. In this sense, natural elements such as cotton, hemp fibre, linen, among others, are being used for preparing different products for construction, for manufacturing clothing and footwear. However, most of said materials comprise some non-recyclable element or some non-natural product, or the end product does not present the desired properties.
Therefore, there is a need to provide a natural and organic product that presents improved properties with respect to the products existing in the state of the art, such as greater strength, viscosity and compaction, such that they allow improved moulding of the board and therefore better use of the end product.

### Brief description of the invention.

The present invention solves the problems of the state of the art given that it provides a mixture for preparing boards with high-compaction and high-strength.

Therefore, in a first aspect, the present invention relates to a mixture comprising natural coconut husk coir particulate and/or balsa wood particulate and/or ground algae and an adhesive (hereinafter mixture of the present invention).

In a particular embodiment, the natural coconut husk coir and balsa wood and/or ground algae particles comprises a size comprised between 0.01-10 mm. In a more particular embodiment, the ground algae particles comprise a size of between 0.5-4 mm.

In another particular embodiment, the mixture of the present invention comprises additives.

In the present invention, additives relate to any component providing or improving at least one property of the mixture such as thickeners, dyes, binders, etc. More preferably, the additives are natural additives.

In another particular embodiment, the mixture of the present invention comprises cork.

In a particular embodiment, the adhesive of the mixture of the present invention is a natural polymer adhesive. Preferably, the adhesive of the present invention is a polyethylene-based adhesive; preferably, the adhesive of the present invention is latex vinyl glue.

In a particular embodiment, the mixture of the present invention comprises:
- 0-90 % by weight of natural coconut husk coir,
- 0-95 % by weight of balsa wood,
- 0-92 % by weight of algae,
- 8-10 % by weight of adhesive.

In a second aspect, the present invention relates to a construction board (hereinafter board of the present invention) comprising the mixture of the present invention.

In a third aspect, the present invention relates to a method for preparing the mixture of the present invention, (hereinafter method of the present invention) comprising the following steps:
a) grinding the natural coconut husk coir and/or balsa wood and/or algae until obtaining a particle size comprised between 0.01-10 mm,
b) dehydrating the natural coconut husk coir and/or balsa wood and/or algae until obtaining a degree of moisture comprised between 5-10 %.
c) mixing the natural coconut husk coir and/or balsa wood and/or ground algae particles with the adhesive.

In a preferred embodiment, natural coconut husk coir and/or balsa wood and/or algae in the form of powder are added to the mixture of step c).

In a preferred embodiment, dehydrating step b) is performed prior to grinding step a).

In another preferred embodiment, cork is added to the mixture of step a).

In another aspect, the present invention relates to a method for preparing the board of the present invention comprising the method for preparing the mixture of the present invention and a moulding step by means of applying between 20-80 bar pressure and 100-200 °C for 5-15 minutes.

### Detailed description of the invention

### Example 1: preparation of the mixture of the present invention from natural coconut husk coir and balsa wood

First, mixing of the components of the mixture was performed as follows:
- 30 % by weight of ground coconut with a particle size comprised between 0.01-10 mm,
- 60 % by weight of ground balsa wood with a particle size comprised between 0.01-10 mm.

Next, dehydration of the preceding mixture was performed; in this case, dehydration was carried out by means of drying in a greenhouse for 12 to 24 hours until a degree of moisture comprised between 5-10 % was obtained; however, dehydration can be carried out under heating or any method known to a person skilled in the art. Once dehydration ended, 10 % by weight of glue adhesive was added and moulding was performed by means of applying between 20-80 bar pressure and 100-200 °C for 5-15 minutes.

### Example 2: preparation of the mixture of the present invention from natural coconut husk coir

First, natural coconut husk coir at a percentage of 90 % by weight with a particle size comprised between 0.01-10 mm was prepared. Next, dehydration of the preceding mixture was performed by means of drying in a greenhouse for 12-24h until a degree of moisture comprised between 5-10 % was obtained. Once dehydration ended, 10 % by weight of glue adhesive was added and moulding was performed by means of applying between 20-80 bar pressure and 100-200 °C for 5-15 minutes.

### Example 3: preparation of the mixture of the present invention from balsa wood.

First, the balsa wood at a percentage of 92 % by weight with a particle size comprised between 0.01-10 mm was prepared. Next, dehydration of the preceding mixture was performed by means of drying in a greenhouse for 12-24h until a degree of moisture comprised between 5-10 % was obtained. Once dehydration ended, 8 % by weight of glue adhesive was added and moulding was performed by means of applying between 20-80 bar pressure and 100-200 °C for 5-15 minutes.

### Example 4: preparation of the mixture of the present invention from natural coconut husk coir and balsa wood and cork

Mixing of the components of the mixture was performed as follows:
- 30 % by weight of ground coconut with a particle size comprised between 0.01-10 mm,
- 40 % by weight of ground balsa wood with a particle size comprised between 0.01-10 mm,
- 20 % by weight of cork.

Next, dehydration of the preceding mixture was performed; in this case, dehydration was carried out by means of drying in a greenhouse for 12-24h until a degree of moisture comprised between 5-10 % was obtained.

Once dehydration ended, 10 % by weight of glue adhesive was added and moulding was performed by means of applying between 20-80 bar pressure and 100-200 °C for 5-15 minutes.

### Example 5: preparation of a board from a mixture of natural coconut husk coir and balsa wood and cork.

The mixture obtained in example 4 was taken to a mould and a pressure of 20-80 bar was applied at a temperature of 100-200 °C for 5-15 minutes, a board being obtained with a thickness comprised between 5 and 50 mm.

### Example 6: Preparation of the mixture of the present invention from ground algae.

First, the ground algae were prepared; to that end, algae from the Mediterranean Sea washed with abundant water were used; preferably, washing was performed in a rotary system to also remove sand and other impurities. Once the washing phase ended, drying of the algae was performed; to that end, drying was performed in a greenhouse for 12-48 hours until a degree of moisture comprised between 5-10 % was obtained; however, drying can be carried out under heating or any drying method known to a person skilled in the art. Lastly, the algae were ground until obtaining particles of a size comprised between 0.5-4 mm.

Once the ground algae were obtained, they were mixed with glue adhesive in the following proportions:
- 92 % by weight of ground algae and,
- 8 % of glue adhesive.

Next, moulding was performed by means of applying between 20-80 bar pressure at a temperature of 100-200 °C for 5-15 minutes.

### Example 7: Preparation of the mixture of the present invention from natural coconut husk coir and balsa wood and ground algae

Prior to preparing the mixture, the ground algae were prepared; to that end, algae from the Mediterranean Sea washed with abundant water were used; preferably, washing is performed in a rotary system. Once sand and other impurities were removed, drying of the algae was performed; to that end, drying was performed in a greenhouse for 12-48 hours until a degree of moisture comprised between 5-10 % was obtained; however, drying can be carried out under heating or any drying method known to a person skilled in the art. Lastly, the algae were ground until obtaining particles of a size comprised between 0.5-4 mm.

Moreover, the following components of the mixture were mixed as follows:
- 30 % by weight of ground coconut with a particle size comprised between 0.01-10 mm,
- 40 % by weight of ground balsa wood with a particle size comprised between 0.01-10 mm.

Once said components were mixed, dehydration of the preceding mixture was performed; in this case, dehydration was carried out by means of drying in a greenhouse for 12-24h until a degree of moisture comprised between 5-10 % was obtained.

Next, the ground algae were mixed with the mixture of coir and weight of balsa wood in the following percentages:
- 30 % by weight of ground coconut with a particle size comprised between 0.01-10 mm,
- 40 % by weight of ground balsa wood with a particle size comprised between 0.01-10 mm,
- 22 % of ground algae

Lastly, 8 % by weight of glue adhesive was added and moulding was performed by means of applying between 20-80 bar pressure and 100-200 °C for 5-15 minutes.

### Example 8: Preparation of a board from a mixture of natural coconut husk coir and balsa wood and algae.

The mixture obtained in example 6 was taken to a mould and a pressure of 20-80 bar was applied at a temperature of 100-200 °C for 5-15 minutes, a board being obtained with a thickness comprised between 5 and 50 mm.

## Claims

1. A mixture comprising natural coconut husk coir particulate and/or balsa wood particulate and/or ground algae and an adhesive, wherein the natural coconut husk coir particle and/or the balsa wood particle and/or the algae particles comprise a size of between 0.01-10 mm.

2. The mixture according to claim 1, wherein the mixture comprises additives.

3. The mixture according to any of claims 1-2, wherein the mixture comprises cork.

4. The mixture according to any of claims 1-2, wherein the ground algae particles comprise a size of between 0.5-4 mm.

5. The mixture according to any of the preceding claims, wherein the adhesive is a natural polymer adhesive.

6. The mixture according to any of the preceding claims, comprising:
- 0-90 % by weight of natural coconut husk coir,
- 0-95 % by weight of balsa wood,
- 0.92 % by weight of ground algae,
- 8-10 % by weight of adhesive.

7. A construction board comprising a mixture according to any of claims 1-6.

8. A method for preparing a mixture according to any of claims 1-6, comprising the following steps:
a) grinding the natural coconut husk coir and/or balsa wood and/or ground algae particles until obtaining a particle size comprised between 0.01-10 mm,
b) dehydrating the natural coconut husk coir and/or balsa wood and/or ground algae particles,
c) mixing the natural coconut husk coir and/or balsa wood and/or ground algae particles with the adhesive.

9. The method according to claim 8, wherein step b) is performed prior to step a).

10. The method according to any of claims 8-9, wherein natural coconut husk coir and/or balsa wood and/or algae in the form of powder are added to the mixture of step c).

11. The method according to any of claims 8-10, wherein cork is added to the mixture of step a).

12. The method for preparing a board according to claim 7, comprising the method for preparing a mixture according to any of claims 8-11 and a moulding step by means of applying between 20-80 bar pressure and 100-200 °C for 5-15 minutes.
